

## UNITED STATES PATENT OFFICE

2,582,958

DETERGENT OIL COMPOSITION AND THE  
METHOD FOR ITS PREPARATIONElmer W. Brennan and Norman D. Williams, Chi-  
cago, Ill., assignors to The Pure Oil Company,  
Chicago, Ill., a corporation of OhioNo Drawing. Application October 16, 1948,  
Serial No. 55,008

18 Claims. (Cl. 260—399)

This invention relates to lubricants and, more particularly, to lubricants having detergent qualities. Specifically, it concerns the method of preparing a new additive for enhancing the detergent characteristics of an oil.

It is a fundamental object of the instant invention to provide a new method of preparing a phosphorized-sulfurized fatty additive having enhanced detergent qualities and containing amounts of metals substantially greater than it has previously been possible to incorporate into the additive.

It is a further object of the invention to provide a new sulfurized-phosphorized detergent lubricating composition containing phosphorus, sulfur and more than one metal.

It is a further object of the invention to provide a new method of preparing sulfurized-phosphorized lubricating oil compositions containing detergent metals.

It is a further object of the invention to provide a method of incorporating a relatively large amount of a detergent metal into a sulfurized-phosphorized lubricating oil additive concentrate.

Other objects and advantages of the invention will in part be obvious and in part appear hereinafter.

We have discovered that an improved lubricating oil additive can be prepared if a fatty material, for example, oleic acid, is first neutralized with a metallic hydroxide or oxide, preferably one which imparts a specific desired property to the additive, then reacted with a phosphorizing-sulfurizing reagent until the reaction is complete, and any functional group produced by the phosphorizing-sulfurizing reagent subsequently reacted with the same or a different metal oxide or hydroxide, thereby to give a compound which has valuable characteristics, the chief of which are its detergent qualities and high metal content.

Typical fatty materials which can be used in our process include fatty acids having about 12 to 30 carbon atoms or more and also having a functional group reactive with a sulfide of phosphorus, such as hydroxy stearic, oleic, ricinoleic acids, oxidized petroleum hydrocarbons containing both hydroxy and olefinic acids and fatty acid mixtures derived from natural oils, such as corn-seed, rapeseed, linseed, sperm and castor oils. The natural oils which are the sources of these various fatty acids themselves are also useful starting materials.

The materials useful for neutralization purposes may be any which will put into the com-

1  
2  
ound a metal which will impart desirable properties and thus would include the metals, oxides, hydroxides and carbonates.

The purpose of using the oxide or the hydroxide of a metal in the saponification reaction or subsequent neutralization is to introduce metal into the fatty material used as the starting material. Where the oxide or hydroxide is soluble in water, theoretically at least, an aqueous solution thereof could be used, but inasmuch as the temperatures involved in the saponification reaction are such that water is normally allowed to distill off, the use of aqueous solutions is avoided. Similarly, where a high molecular weight fatty acid, such as oleic is used as the starting material, the initial saponification could be carried out by reaction of the acid with the metal. However, as noted, convenience dictates the use of an oxide or a hydroxide. In general the oxides and hydroxides of the saponifying metals can be used interchangeably. Thus, in the saponification of the fatty material or the subsequent neutralization of the phosphorized-sulfurized salt, the active ingredient in the reaction is the metal oxide and those cases in which the hydroxide is used are the full equivalent thereof, but the hydroxide is used as a matter of convenience. Thus, barium imparts good detergency to the product; zinc imparts good anti-oxidant properties. An additive having good detergent and anti-oxidant qualities can, therefore, be made by neutralizing the fatty starting material with barium oxide or hydroxide, sulfurizing and phosphorizing with any phosphorizing and sulfurizing agents, such as phosphorus, sulfur, their oxides and chlorides, phosphorus sesquisulfide and phosphorus pentasulfide, and finally neutralizing with zinc oxide or hydroxide. Thus, to impart specific detergent and anti-oxidant properties to the additive, various combinations of neutralizing materials can be used, such as hydroxides and oxides of zinc, barium, calcium, strontium, magnesium, tin, lead, nickel, and cobalt as well as various amines.

45 The following examples illustrate a few typical preparations:

Example I.—Two hundred (200) grams of oleic acid dissolved in 800 grams of 160/180 viscosity Mid-Continent solvent refined oil was heated with agitation to 275° to 300° F. The principal quality desired of the diluent oil or reaction medium is that it should be inert and unreactive with the phosphorizing and sulfurizing agents used in the reaction. Certain hydrocarbon solvents like toluene are useful in the operation because they are free of reactive materials. To this

solution there was added 27.6 grams of calcium hydroxide of 95 per cent purity, thereby completely neutralizing the oleic acid. All of the water formed in the neutralization reaction was evaporated and the temperature was lowered to 240° F. At this point, 14 grams of phosphorus sesquisulfide (7 per cent by weight on the basis of oleic acid) was added. During the addition of the phosphorus sesquisulfide, air was passed into the reaction mixture at the rate of 45 cubic feet per hour in order to maintain a temperature of 250° F. without employing external heat. Under these conditions, the phosphorization-sulfurization reaction is quite exothermic and the technique of aerating a mixture during reaction thereof reduces or eliminates the necessity for the application of external heat. Within a period of about 25 minutes, the reaction was completed as evidenced by the cessation of fuming of the reaction mixture. It is also to be noted that upon completion of the phosphorization-sulfurization reaction, the temperature sustained by the heat of the reaction drops off. This characteristic of the reaction can be used as a good index of the time of completion. After reaction of the neutralized oleic acid with phosphorus sesquisulfide, the temperature was raised to 275° to 300° F. and 54 grams of barium hydroxide octahydrate was added to the solution. Heating was continued for half an hour after the final addition of the hydroxide. The product was filtered to remove solids and the composition by weight of the filtrate was as follows:

| Actual (By analysis) | Theoretical |
|----------------------|-------------|
| Per Cent Ba—2.19     | 2.23        |
| Per Cent Ca—1.15     | 1.35        |
| Per Cent S—0.52      | 0.58        |
| Per Cent P—0.67      | 0.75        |

When expressed in terms of active components, the composition appears as follows:

| Actual                    | Theoretical |
|---------------------------|-------------|
| Per Cent Ba—9.27          | 9.33        |
| Per Cent Ca—4.87          | 5.65        |
| Per Cent S—2.20           | 2.41        |
| Per Cent P—2.83           | 3.11        |
| Per Cent Oleic Acid—80.83 | 79.50       |

From the analysis reported above, it can be readily seen that some calcium was lost. It is entirely possible that some barium displaced the calcium but, however, the magnitude of the barium content is such that it is apparent it would have been necessary to displace 2.71 per cent calcium to introduce 9.27 per cent barium into the molecule. Since only 0.78 per cent calcium was lost from the theoretical value of 5.65 per cent, the barium must have entered the molecule at another point, viz., the thiophosphorus group. Some of the loss of calcium was undoubtedly due to hydrolysis during the second neutralization and/or removal in the course of the sulfurizing-phosphorizing reaction.

Sufficient of the material was blended with a Mid-Continent solvent refined oil SAE-10, to give a total metal content of 0.27 per cent. The finished blend gave no evidence of separation after storage of samples at room temperature and 30° F. for 10 days.

*Example II.*—Following the procedure outlined in Example I, calcium oleate was prepared and to it 14 grams of phosphorus pentasulfide per hundred grams of oleic acid was added and re-

acted at about 300° F. for two hours. At the end of this time, there was no evolution of hydrogen sulfide, indicating that the reaction was complete. At this point 37 grams of barium hydroxide octahydrate was added while the reaction mixture was held at 275° to 300° F. Heating was continued for a half hour after the final addition of the hydroxide. Two per cent filter aid was then added, the product was filtered to remove solids and analyzed. The composition was as follows:

| Actual (By Analysis) | Theoretical |
|----------------------|-------------|
| Per Cent Ba—1.47     | 1.52        |
| Per Cent Ca—1.12     | 1.34        |
| Per Cent P—0.78      | 0.64        |
| Per Cent S—1.55      | 1.90        |

In terms of active ingredients, the composition would be:

| Actual                    | Theoretical |
|---------------------------|-------------|
| Per Cent Ba—6.15          | 6.23        |
| Per Cent Ca—4.69          | 5.50        |
| Per Cent P—3.26           | 3.30        |
| Per Cent S—6.49           | 7.50        |
| Per Cent Oleic Acid—79.41 | 77.47       |

One of the tests of the stability of any hydrocarbon product is its resistance to deterioration in storage. For example, samples of a finished blend consisting of Mid-Continent solvent refined oil and the above additive showed no evidence of deterioration after prolonged storage at room temperature and 30° F.

The composition has the advantage that it can be made to show a high degree of detergency by incorporating into the starting material any of a wide variety of metals, namely, barium, strontium, other alkaline earth materials, and also tin, zinc, lead and nickel.

By the proper choice of metals, an additive possessing specific different functions in a single molecule or composition can be prepared. For example, if barium oleate is treated with a sulfide of phosphorus and then the thiophosphorus material neutralized with barium oxide or hydroxide, the product will have a high degree of detergency and a metal content in excess of the stoichiometric equivalent of the starting acid. However, if zinc oxide were to be used in place of barium hydroxide to neutralize the thiophosphorus material, a two-purpose additive as a single compound would be prepared. That is, the barium soap portion of the molecule would impart good detergency properties, whereas the zinc-sulfur-phosphorus would impart anti-oxidant properties. Thus, a detergent additive made in accordance with the invention can contain the same combination of ingredients, but can display different properties depending upon the order in which they were combined. In the preparation of a series of additives, it was found that zinc, for example, could be used in either the first saponification step or in the subsequent neutralization and that the effect of moderating the viscosity increase of the oil blend after use was retained.

This phase of the composition is illustrated by the following compounds made in accordance with the procedure described:

- No. 1—Barium salt of barium oleate.
- No. 2—Zinc salt of barium oleate.
- No. 3—Barium salt of zinc oleate.

75 Composition No. 1 is the barium salt of sulfur-

ized-phosphorized barium oleate; composition No. 2 is the zinc salt of sulfurized-phosphorized barium oleate; and composition No. 3 is the barium salt of sulfurized-phosphorized zinc oleate. The compositions, though similar in the nature of ingredients used, differ in method of preparation and possess characteristics which would differ in kind and degree. Double lead salts corresponding to the above compounds might be used in extreme pressure lubricants to increase the load carrying capacity.

There is a limit to the amount of metal which can be added in the second neutralization reaction carried out in accordance with the process described. Thus, referring to Example II, when 1.55 per cent barium was added to the compound, a moderately viscous liquid product was obtained. When the percentage of barium was increased to 2, a very viscous product resulted. When the percentage was increased to a level between 2.00 and 2.25 per cent, the product gelled. This gel is not soluble in Mid-Continent solvent refined SAE-10 oil to the extent needed to give approximately 0.27 per cent metal in the composition. Using a product of the highest metal concentration which is acceptable on the basis of solubility, a material containing 28 per cent barium (this figure being based on active ingredients) is derived. Similarly, there are limiting percentages, above which gel formation will take place for each metal or combination of metals.

As the initial fatty acid reagent, any compound which has a carboxyl group plus a functional group which is reactive with a sulfide of phosphorus can be used. Examples of such possible compounds are hydroxy fatty acids, such as hydroxy stearic acid, olefinic materials, or oxidized petroleum fractions which contain both hydroxy acids and keto acids. It is not necessary that the starting material be a free acid for any of the natural fats or oils which give an acid containing the desired functional group can be used. Thus, the various oils, fats and waxes, such as sperm oil, castor oil, linseed oil, rapeseed oil; fats containing unsaturated acids, degras, and the like can be employed.

An example of another composition prepared in accordance with the invention is the following:

*Example III.*—Six hundred (600) grams of neutral degras, commonly known as wool grease or wool wax, was heated to 300° to 325° F. with stirring. The wool fat was then saponified with 150 grams of barium hydroxide octahydrate. As the saponification proceeded, the reaction mixture became extremely viscous. After the final addition of the hydroxide had been made, the temperature was dropped to 230° F. and 45 grams of phosphorus sesquisulfide added. Air was passed into the reaction mixture at a rate sufficient to maintain a temperature of 240° F. without the use of external heat. Within a few minutes, the contents of the reaction flask became more fluid. When the sulfide had been completely reacted as evidenced by a cessation of fuming and a drop in temperature, in spite of a more rapid flow of air, 1200 grams of 160/180 neutral Mid-Continent solvent refined oil was added to the reaction product. When the complete solution had taken place, 168 grams of barium hydroxide octahydrate was added at 275° to 300° F. to neutralize the sulfur-phosphorus acidity. The filtered product contained 7.0 per cent barium determined by the sulfated residue method. This figure exceeded the theoretical one of 6.4 per cent, but the discrepancy can be attributed to experimental error.

The detergent qualities of the composition were tested for 120 hours under the Caterpillar diesel L-1 test procedure (CRC designation L-1-545). Though normally the Caterpillar diesel L-1 test lasts 480 hours, an approximate measure of the effectiveness of the detergent can be determined in 120 hours. That is, the detergency of an oil can be measured on the degree of engine cleanliness maintained in 120 hours of the test.

10 The following examples summarize the results of several tests conducted to evaluate the detergent composition:

*Example 1.*—A blend of an SAE-30 Mid-Continent solvent refined oil containing 0.5 per cent 15 of an anti-corrosion additive known commercially as "Santolube 394-C" was subjected to 120 hours of test following the Caterpillar L-1 diesel test procedure and evaluated for detergency on the basis of an examination of the ring grooves, 20 lands and skirt of the engine pistons after the test. The ring grooves showed heavy carbon and black varnish deposits, the lands showed relatively heavy and medium deposition of black varnish and the skirt showed varnish above the 25 pin boss and on the side opposite from the thrust side. In view of the condition of the parts of the piston, the over-all rating of the oil was such that the oil was considered a failure.

*Example 2.*—A composition consisting of an 30 SAE-30 Mid-Continent solvent refined oil including 1 per cent of "Santolube 394-C" as a corrosion inhibitor and 0.27 per cent by weight of metal in the form of the double salt additive was subjected to 120 hours of test following the 35 Caterpillar L-1 diesel test procedure. The additive used was the barium salt of zinc oleate made from oleic acid in accordance with the procedure described in Example II, wherein zinc oxide was used to neutralize oleic acid, the product 40 phosphorized and sulfurized and the acidity thus developed neutralized with barium hydroxide. After 120 hours of the Caterpillar L-1 diesel test, the engine was examined for the condition of the ring grooves, lands and skirt. The ring 45 grooves showed light deposits of soft carbon, light deposits of clear varnish and the fourth ring groove was clean. The lands had relatively light coatings of dark varnish and the skirt of the piston was clean. In view of the condition 50 of the ring grooves, lands and skirt, the detergent combination was considered effective in maintaining engine cleanliness.

*Example 3.*—A similar test was conducted 55 using a composition consisting of an SAE-30 Mid-Continent solvent refined oil containing 1 per cent of "Santolube 394-C" and 0.27 per cent by weight of barium from the double barium salt of phosphorized-sulfurized wool grease made in accordance with the procedure described in 60 Example III. After 120 hours of test under the Caterpillar L-1 diesel test procedure, the pistons were examined for their condition. The ring grooves showed a moderately light carbon deposit and a moderate varnish deposit. The lands between the grooves showed light coatings of varnish on only the first, the others being clean. The skirt was clean. On the basis of these results, the detergent combination was effective in maintaining engine cleanliness.

*Example 4.*—A blend consisting of an SAE-30 Mid-Continent solvent refined oil plus 1 per cent of "Santolube 394-C" plus 0.27 per cent by weight of metal obtained by the addition to the blend of the barium salt of the zinc saponified wool 75 grease prepared in accordance with the proce-

dure described in Example III was subjected 120 hours to the Caterpillar L-1 diesel test procedure. This composition is typical of those which can be prepared from a fatty material which has been sulfurized and phosphorized and reacted to form the salt. After the 120 hour run, the ring grooves, lands and skirt of the piston were examined for their condition. Of the ring grooves, only the first showed a slight carbon deposit on the thrust side, the rest was clean. The remaining ring grooves were also clean. The lands had a light varnish coating on a few areas on the first, and the remainder were clean. The skirt was clean. On the basis of these results, the detergent combination was 15 rated exceptionally good.

The "Santolube 394-C" used in the tests reported in the examples is a sulfurized-phosphorized terpene-like material commonly used as an anti-corrosive additive in oils. Its properties are: viscosity at 210° F., 145 SUS; specific gravity, 1.03; phosphorus content, 4.75 per cent; sulfur content, 12.5 per cent.

*Example 5.*—For a reference test, a typical solvent refined oil like those used in Examples 1 through 4, with no additive, was subjected to 120 hours of test in a diesel engine operated in accordance with the L-1 diesel test procedure used in Examples 1 through 4. Following the test, the pistons were examined for their condition in order to provide a basis for rating the oil. The crown was evenly coated with a film of hard carbon and varnish. Of the ring grooves, the top ring had a very heavy carbon and varnish deposit. The second, third and fourth rings had a heavy black varnish deposit. Though the skirt of the piston appeared clean, it had some amber varnish thereon which alone is sufficient to rate the oil poor. The over-all rating of the oil of the test was considered poor and, of course, 10 the oil failed.

From these several examples, it can be seen that the detergent properties of the material can be varied by adopting different combinations of metals and fatty starting materials. In general, the alkaline earth metals when used as saponifying agents in the fatty material will impart good detergent properties to the oil. Barium is found to be the preferable alkaline earth metal to use because it appears to enhance detergent properties to the greatest extent. Combinations of the metals, such as barium and zinc, and zinc and barium with the same fatty materials can be used, for properties can be altered according to the order in which the metals are reacted with the fatty material. By using the same metal for the saponification and subsequent neutralization, a detergent having a very high concentration of a single metal can be produced. Thus, barium, which is one of the better detergent metals, can be added to a composition to give a very high concentration of the metal. Two different metals can be used to impart slightly different properties or to balance properties and still to add to the composition a large concentration of metal. This is best exemplified by Example 4 given above wherein the barium salt of wool grease phosphorized-sulfurized zinc compound was used and found to have exceptionally good detergent properties.

It will be understood from the preceding examples that the composition contemplated is one which contains an amount of metal which exceeds that which is necessary for the neutralization of the carboxyl group of the fatty material

employed. Thus, a salt of any fatty acid having 12 or more carbon atoms, for example, and also containing a functional group reactable with a phosphorus sulfide, can be used as a starting material and subjected to sulfurization and phosphorization. In general, any phosphorizing-sulfurizing reagent is useful in the process, for it is not the particular reagent which is important in deriving the final product, but it is the product which has its functional group reacted with the phosphorus and the sulfur.

Thus, although the invention has been described with only a limited number of examples, they have been chosen to illustrate the several ramifications of the composition and the method of incorporating a large amount of metal therein and are to be considered as illustrative of the scope and not restrictive thereof.

What is claimed is:

1. The method of preparing a composition suitable as a lubricant additive comprising preparing a salt of wool grease and a metal selected from the group consisting of zinc, barium, calcium, strontium, magnesium, tin, lead, nickel, and cobalt, reacting the salt with a sulfide of phosphorus at a temperature between 200 and 300° F. for a period of time sufficient to sulfurize and phosphorize the salt, and neutralizing the sulfurized-phosphorized salt with a basic compound of a metal of the group consisting of zinc, barium, calcium, strontium, magnesium, tin, lead, nickel, and cobalt, the total amount of metal reacted to form the resulting product being substantially in excess of the amount required to saponify the wool grease.

2. Method in accordance with claim 1 in which the metal used in preparing the salt and for neutralizing the sulfurized-phosphorized salt is barium.

3. Method in accordance with claim 1 in which the metal used in preparing the salt is barium and the metal used for neutralizing the sulfurized-phosphorized salt is zinc.

4. Method in accordance with claim 1 in which the metal used in preparing the salt is zinc and the metal used for neutralizing the sulfurized-phosphorized salt is barium.

5. Method in accordance with claim 1 in which the salt of wool grease is reacted with phosphorus sesquisulfide at a temperature of about 240° F. while bubbling air through the mixture at a rate sufficient to maintain the aforesaid temperature without external heating until the exothermic reaction is completed.

6. A composition of matter useful as a lubricating oil additive to enhance detergent properties of mineral lubricating oils, said composition being a metal salt of fatty material having 12 to 30 carbon atoms in the acid radical and a metal from the group consisting of zinc, barium, calcium, strontium, magnesium, tin, lead, nickel, and cobalt, which salt has been chemically combined with a sulfide of phosphorus at a temperature of 200-300° F. and then neutralized with a basic compound of a metal from the group consisting of zinc, barium, calcium, strontium, magnesium, tin, lead, nickel, and cobalt, said composition containing an amount of combined metal substantially in excess of the amount required to saponify the fatty material.

7. In the method of preparing a lubricating oil additive, the steps of reacting a salt of a metal from the group consisting of zinc, barium, calcium, strontium, magnesium, tin, lead, nickel, 75 and cobalt and a fatty acid having from 12 to 30

carbon atoms in the molecule and a functional group reactive with a sulfide of phosphorus, with a sulfide of phosphorus and subsequently neutralizing the phosphorized-sulfurized material with a basic compound of a metal from the group consisting of zinc, barium, calcium, strontium, magnesium, tin, lead, nickel, and cobalt, the weight per cent of metal in the neutralized material being substantially greater than that in said salt.

8. In the method of preparing a lubricating oil additive, the steps of forming a salt of a metal from the group consisting of zinc, barium, calcium, strontium, magnesium, tin, lead, nickel, and cobalt and a fatty acid having from 12 to 30 carbon atoms in the molecule and a functional group reactive with a sulfide of phosphorus, reacting said salt with a sulfide of phosphorus and subsequently neutralizing the phosphorized-sulfurized material with a basic compound of a metal from the group consisting of zinc, barium, calcium, strontium, magnesium, tin, lead, nickel, and cobalt, the weight per cent of metal in the neutralized material being substantially greater than that in said salt.

9. The method in accordance with claim 7 in which the sulfide of phosphorus and metal salt are reacted at a temperature in the range of about 200 to 300° F. and the sulfurized-phosphorized material is neutralized at a temperature in the range from 250° F. to about 350° F.

10. Method in accordance with claim 7 in which the salt is a barium salt, the sulfide of phosphorus is phosphorus-sesquisulfide and the neutralizing agent is a basic zinc compound.

11. Method in accordance with claim 10 in which the salt is barium oleate.

12. Method in accordance with claim 7 in which the salt is a zinc salt, the sulfide of phosphorus is phosphorus sesquisulfide and the neutralizing agent is a basic barium compound.

13. Method in accordance with claim 12 in which the salt is zinc oleate.

14. Method in accordance with claim 7 in which the salt is a barium salt, the sulfide of phosphorus is phosphorus sesquisulfide and the neutralizing agent is a basic barium compound.

15. Method in accordance with claim 14 in which the salt is barium oleate.

16. A composition in accordance with claim 6 which is the barium salt of wool grease chemically reacted with phosphorus sesquisulfide and subsequently neutralized with a basic barium compound.

17. A composition in accordance with claim 6 which is the barium salt of wool grease chemically reacted with phosphorus sesquisulfide and subsequently neutralized with a basic zinc salt.

18. A composition in accordance with claim 6 which is the zinc salt of wool grease chemically reacted with phosphorus sesquisulfide and subsequently neutralized with a basic barium salt.

ELMER W. BRENNAN.  
NORMAN D. WILLIAMS.

## REFERENCES CITED

30 The following references are of record in the file of this patent:

## UNITED STATES PATENTS

| Number        | Name                  | Date         |
|---------------|-----------------------|--------------|
| 35 Re. 22,849 | Williams et al. ----- | Mar. 4, 1947 |
| 2,420,274     | Williams et al. ----- | May 6, 1947  |
| 2,441,587     | Musselman -----       | May 18, 1948 |